

1

3,778,377

**PROTECTING METAL DURING ACID CONTACT**  
Herbert D. Clark, Burbank, Calif., assignor to Universal  
Oil Products Company, Des Plaines, Ill.  
No Drawing. Filed Oct. 6, 1971, Ser. No. 187,120  
Int. Cl. C02b 5/06

U.S. Cl. 252—82

7 Claims

**ABSTRACT OF THE DISCLOSURE**

Protecting metal during contact with acid by incorporating an inhibitor mixture of a polyaminomethylenephosphonate and an N,N'-dicycloalkyl-thiourea. The inhibitor mixture is used in descaling, acid cleaning, acid pickling, etc.

**BACKGROUND OF THE INVENTION**

During acid cleaning of metal, extreme care must be observed in order to protect the metal against being eaten away by the acid. For example, in removing scale deposits from metal surfaces, the delicate task requires removal of the scale but not injuring the metal proper. Similarly, in other acid cleaning operations, it is important to protect the metal against excessive destruction by the acid. The same precautions must be observed in acid pickling operations, as well as in other industrial acid cleaning steps.

**DESCRIPTION OF THE INVENTION**

The present invention provides a novel inhibitor composition which is added to the acid solution and serves to protect the metal. A particular application is the removal of scale deposits in boilers used to generate steam, in cooling water systems or in other operations in which scale deposits are formed by the polyvalent ions contained in the water. The deposits generally are salts such as calcium sulfate, calcium carbonate, barium salts, sodium salts, etc. As another advantage to the present invention, scale formation is inhibited by acid treatment effected in accordance with the present invention. Scale deposits also are a problem in oil producing equipment. Still other applications relate to acid cleaning, acid pickling, etc.

In one embodiment the present invention relates to a mixture of a polyaminomethylenephosphonate and an N,N'-dicycloalkyl-thiourea.

In a preferred embodiment the polyaminomethylenephosphonate is in a major concentration and may comprise from about 55% to about 95% by weight and the N,N'-dicycloalkyl-thiourea may be in a concentration of from about 5% by weight to about 45% by weight. However, in another embodiment, these concentrations may be within the range of from about 50% to about 99% of the former and from about 1% to about 50% by weight of the latter. These percentages are on an active ingredient basis and exclusive of other components contained in the composition.

In another embodiment the present invention relates to the method of acid cleaning metal surfaces which comprises contacting said metal surfaces with an acid solution containing the novel composition hereinbefore set forth.

In a specific embodiment the present invention relates to a method of removing scale in boilers used to generate steam from water, which comprises treating the same with an aqueous acid solution containing the inhibitor composition hereinbefore set forth.

While the polyaminomethylenephosphonate has been proposed heretofore for use in inhibiting precipitation and scale formation, as described in U.S. Pat. 3,336,221, it now has been found that surprisingly improved results are obtained when the polyaminomethylenephosphonate is used in admixture with the N,N'-dicycloalkyl-thiourea. As will be shown by the appended examples, a synergistic

2

effect is obtained. This is a surprising result because, while the dicycloalkyl-thiourea has been proposed heretofore for use as an acid inhibitor, it has not been proposed for use to remove scale. Thus, the synergistic effect obtained when using these components in admixture would not be expected.

As hereinbefore set forth, one component of the novel composition of the present invention is a polyaminomethylenephosphonate. Numerous polyaminomethylenephosphonates are described in U.S. Pat. 3,336,221 and are incorporated herein by reference. The polyaminomethylenephosphonate may be illustrated by the following structure:



where  $m$  is 1 to 3 and  $n$  is 3 to 15. Also included are the ammonium or alkaline metal salts thereof, or mixtures of these. In a preferred embodiment  $n$  in the above structure is from about 8 to about 12. Typical properties of a preferred polyaminomethylene phosphonate, in which  $m$  in the above structure is 2 and  $n$  is about 10 is stated to be substantially as follows.

TABLE 1

| Item:                     | Description |
|---------------------------|-------------|
| Phosphorus, wt. percent   | 10.         |
| pH                        | 1.0.        |
| Density, pounds/gallon    | 10.5.       |
| Viscosity at 20° C., cps. | 96.         |
| Color                     | Dark amber. |
| Molecular weight          | About 1200. |

The polyaminomethylenephosphonate will be utilized as such or prepared as a solution or dispersion in a suitable solvent, emulsifier, dispersant or the like, which may be selected from those hereinafter set forth.

Another component of the inhibitor composition of the present invention is N,N'-dicycloalkyl-thiourea and particularly N,N'-dicyclohexyl-thiourea. Other dicycloalkyl derivatives contain 3 to 5 or 7 to 12 carbon atoms in the cycloalkyl ring. The N,N'-dicycloalkyl-thiourea preferably is utilized as a 5 to 25% by weight solution or suspension in a water soluble solvent, emulsifier, dispersant or the like.

Any suitable water soluble solvent, emulsifier, dispersant or the like may be used and may be selected from one or more of the following: (1) alcohols including methanol, ethanol, propanol, butanol, etc., (2) glycols including ethylene glycol, diethylene glycol, propylene glycol, di-propylene glycol, dimethylethylene glycol, trimethyldiethylene glycol and higher molecular weight polyethylene glycols or polypropylene glycols, (4) ketones including acetone, methylethyl ketone, diethyl ketone, methylpropyl ketone, ethylpropyl ketone, dipropyl ketone, etc., (5) polyoxyethylene ether, polyoxypropylene ether, methoxy polyoxyethylene glycol, etc., (6) dimethylformamide, dimethylacetamide, diethylacetamide, dipropylacetamide, dimethylpropionamide, diethylpropionamide, etc., or (7) mixtures thereof. A particularly preferred mixture used with the dicyclohexyl-thiourea is from about 5% to about 20% dicyclohexyl-thiourea, from about 40% to about 80% by weight of N,N-dimethylacetamide and from about 5% to about 30% by weight of polyoxyethylene and/or polyoxypropylene derivative. The polyethylene glycols

preferably have a molecular weight of from about 150 to about 1000 and more particularly from about 180 to about 800. The particular compound or compounds to be used will be selected with reference to the particular mixture of polyaminomethylene phosphonate and dicycloalkyl-thiourea and the particular acid employed, as well as the particular type of metal surface to be cleaned. The phosphonate and/or thiourea on an active ingredient basis may be in a concentration of from about 5% to about 95% by weight and preferably from about 8% to about 60% by weight.

In still another embodiment the inhibitor composition may contain a color indicator to permit visual observation of loss of potency of the inhibitor composition. For example, Methyl Violet may be included in the composition to indicate loss of potency when the color changes from violet to reddish. The amount of Methyl Violet will be sufficient for the purpose and may be used in an amount of from about 0.5 to about 10% by weight of the inhibitor composition, based on active ingredients, although lower or higher concentrations may be used as desired. It is understood that other suitable color indicators may be employed.

In a preferred method, the inhibitor mixture, with or without color indicator, is first prepared and then added to an aqueous solution of the acid. The specific amount of inhibitor composition to be included in the aqueous solution will be selected with reference to the particular use thereof. For example, when used for descaling, the inhibitor composition will be determined with regard to the amount and type of scale to be removed. The concentration of inhibitor composition may be within the range of from about 0.1 to about 1000 and preferably from about 0.1 to about 100 p.p.m. (parts per million) based on the acid, although lower or higher concentrations may be used as desired. The appended examples illustrate suitable solutions.

As hereinbefore set forth, in one application the inhibitor composition of the present invention is used in acid solutions to remove scale formation in boilers. The scale is formed from water having high concentrations of polyvalent ions, and may comprise one or more of calcium salts, barium salts, magnesium salts, sodium salts, etc., such as the carbonate, sulfate, oxalate, silicate, etc. The scale deposits lead to plugging, pumping difficulties, loss of heat transfer, etc. Similar problems occur in cooling water systems and the removal of the scale is necessary to insure efficient operation. In another application, acid solutions are used to clean metal surfaces including, for example, in acid pickling systems. Regardless of the particular acid treatment, it is important to protect the metal from excessive loss of metal or other impairment thereof.

The acid treatment is effected in conventional manner using any suitable acid, including hydrochloric, sulfuric, phosphoric, etc. These acids treatments are well known in the industry and accordingly need not be described in detail herein. The inhibitor composition is incorporated in the acid solution in any suitable manner.

The following examples are introduced to illustrate further the novelty and utility of the present invention but not with the intention of unduly limiting the same.

#### EXAMPLE I

A series of evaluations was made in the following manner. Zinc strips of equal dimensions and of approximate equal weight of 2 grams were used as the test strips. The acid solution comprised 200 ml. of a 10% distilled water dilution of 15° Baumé commercial muriatic acid. The zinc strips were immersed in the solution for a period of 3 hours at a temperature of 100° F.

The inhibitor components, as indicated below, were mixed with 467.5 grams of 15° Baumé muriatic acid and the mixture diluted to 10% with distilled water.

The zinc strip immersed in the acid solution which contained no inhibitor was completely destroyed, as shown in the following table.

TABLE 2

| Test No. | Inhibitor               | Time, minutes | Weight loss, percent |
|----------|-------------------------|---------------|----------------------|
| 5        | None                    | 120           | 100.00               |
|          | 2 g. PMP                | 180           | 73.34                |
|          | 2 g. DCT <sup>2</sup>   | 180           | 19.37                |
|          | 1 g. PMP 1 g. DCT       | 180           | 1.69                 |
|          | 1.33 g. PMP 0.67 g. DCT | 180           | 5.63                 |
|          | 0.67 g. PMP 1.33 g. DCT | 180           | 35.04                |

10 <sup>1</sup> Polyaminomethylene phosphonate of the structure hereinbefore set forth in which *m* is 2 and *n* is about 10.

<sup>2</sup> N,N'-dicyclohexyl-thiourea.

15 The dicyclohexyl-thiourea used in this example is a commercial product available under the trade name of "Main 33S" and is believed to comprise about 10% by weight of N,N'-dicyclohexyl-thiourea, about 60% by weight of N,N-dimethylacetamide and about 30% by weight of a polyoxyethylene or polyoxypolyethylene derivative of a molecular weight of about 800. The amount of the "DCT" in Table 2 is the mixture of thiourea, dimethylacetamide and the polyoxyethylene derivative.

20 From the data in the above table, it will be seen that the zinc strip immersed in the acid solution, not containing inhibitor, was completely destroyed. On the other hand, it will be noted that the PMP and DCT each separately served to protect the metal to varying degrees. However, it will be seen that the equal weight mixture considerably reduced the weight loss as shown in Test No. 4. A considerable reduction in weight loss was obtained when using the mixture of Test No. 5. When compared to the use of the PMP alone, the mixture used in Test No. 6 resulted in considerable improvement. However, for protecting zinc it is preferred that the PMP and DCT be used in substantially equal amounts for optimum results.

#### EXAMPLE II

25 Another series of evaluations were made in substantially the same manner as in Example I, but using mild steel strips. The steel strips were of equal dimensions and of approximate equal weight of 11 grams. Each strip was immersed in 200 ml. of a 20% distilled water dilution of 15° Baumé commercial muriatic acid for a period of 15 hours at a temperature of 140° F. The additives in the amounts shown in the following table were 30 mixed with 467.5 grams of 15° Baumé muriatic acid and the mixture diluted to 20% with distilled water. The results of these tests are reported in the following table.

TABLE 3

| Test No. | Inhibitor         | Weight loss |
|----------|-------------------|-------------|
| 7        | None              | 7.20        |
| 8        | 2 g. PMP          | 0.62        |
| 9        | 2 g. DCT          | 0.96        |
| 10       | 1 g. PMP 1 g. DCT | 0.54        |

35 55 Here again a synergistic effect was obtained when using the mixture of PMP and DCT as compared to the use of either component alone. While these results are not as startling as compared to the results reported in Example I, a considerable improvement was obtained, ranging from 13% to 83% when compared with the use of PMP or DCT alone.

#### EXAMPLE III

60 65 An inhibitor composition is prepared to comprise equal weight amounts of the sodium salt of amino-tri-(methylphosphonic acid) and the N,N'-dicyclohexyl-thiourea mixture described in Example I. This mixture is used in a concentration of 1 part in 20 parts of aqueous acid solution and the resulting mixture is utilized to clean metal in conventional manner. Here again, the use of the inhibitor composition inhibits eating away of the metal by the acid.

70 75 I claim as my invention:

1. A synergistic mixture of from about 50% to about 99% by weight of polyaminomethylene phosphonate and

from about 1% to about 50% by weight of N,N'-dicycloalkyl-thiourea.

2. The mixture of claim 1 in which said thiourea is N,N'-dicyclohexyl-thiourea.

3. The mixture of claim 1 in which said polyaminomethylenephosphonate is in a concentration of at least 55%.

4. The mixture of claim 2 in which said N,N'-dicyclohexyl-thiourea is prepared as a composition of from about 5% to about 20% by weight of N,N'-dicyclohexyl-thiourea, from about 40% to about 80% by weight of N,N-dimethylacetamide, and from about 5% to about 30% by weight of polyoxyethylene or polyoxypropylene derivative.

5. The method of removing scale from a metal surface in a boiler used to generate steam from water, which comprises treating said surface with an acid solution containing the synergistic mixture of claim 2.

6. The method of cleaning a metal surface by treatment with an acid solution, which comprises adding to the

20 134-3; 252-389, 391, 181, 87, 149  
7. In the acid pickling of metal, the improvement which comprises adding to the acid solution the synergistic mixture of claim 2.

References Cited

UNITED STATES PATENTS

|              |        |            |       |         |
|--------------|--------|------------|-------|---------|
| 3,336,221    | 8/1967 | Ralston    | ----- | 210-58  |
| 3,188,292    | 6/1965 | Pirotte    | ----- | 252-149 |
| 3,260,538    | 7/1966 | Gardner    | ----- | 252-391 |
| 3,440,095    | 4/1969 | Larsonneur | ----- | 134-3   |
| 10 3,669,902 | 9/1970 | Hirner     | ----- | 252-391 |

FOREIGN PATENTS

|         |        |           |       |         |
|---------|--------|-----------|-------|---------|
| 285,284 | 8/1968 | Australia | ----- | 252-391 |
|---------|--------|-----------|-------|---------|

15 GEORGE F. LESMES, Primary Examiner

W. R. DIXON, JR., Assistant Examiner

U.S. Cl. X.R.